

Nov. 27, 1956

M. F. QUAELY ET AL

2,772,227

PROTECTION OF MOLYBDENUM AND TUNGSTEN AT HIGH TEMPERATURES

Filed June 29, 1953

FIG. 1



FIG. 2



FIG. 2

INVENTORS  
MARTIN F. QUAELY  
WM. C. LILLIENDAHL

BY *J. F. Kelly*  
ATTORNEY

1

2,772,227

## PROTECTION OF MOLYBDENUM AND TUNGSTEN AT HIGH TEMPERATURES

Martin F. Quale, Montclair, and William C. Lilliendahl, Mountain Lakes, N. J., assignors to Westinghouse Electric Corporation, East Pittsburgh, Pa., a corporation of Pennsylvania

Application June 29, 1953, Serial No. 364,632

5 Claims. (Cl. 204—32)

This invention relates to readily oxidizable metals and improved means for protecting them against oxidation at elevated temperatures.

The principal object of our invention, generally considered, is to produce articles from refractory readily-oxidizable metals in which oxidation thereof at elevated temperatures is prevented by a complex coating, which is not only firmly adherent, but flexible without peeling from the base material.

Another object of our invention is to protect articles which are constructed of refractory but readily-oxidizable metals, such as molybdenum, tungsten, alloys thereof with each other, and alloys thereof with small proportions of metal of the group consisting of cobalt, nickel and iron, comprising cleaning said articles, and electroplating them with a black chromium-vanadium or chromium-nickel-vanadium complex.

A further object of our invention is the protection of molybdenum and other materials having similar oxidation characteristics with coatings of improved ductility and resistance consisting of black complex chromium base coatings electrolytically applied and including a proportion of vanadium.

Other objects and advantages of the invention will become apparent as the description proceeds.

Referring to the drawing:

Figure 1 is a vertical sectional view of a plating bath which may be used for coating articles in accordance with our invention.

Figure 2 is a transverse sectional view of an article of molybdenum coated or plated with a chromium-vanadium complex.

Figure 3 is a vertical sectional view of a furnace in which articles so plated may be heat treated for improving their characteristics.

There are a number of metals, such as molybdenum, tungsten and alloys thereof, and particularly molybdenum, which have very good and useful properties as to strength, hardness and relatively high melting points, but which are susceptible to oxidation at moderately high temperatures. Molybdenum, for example, starts to oxidize at about 400° C., and at about 700° C. the oxide is not only rapidly formed but is volatile, so that at any temperature thereabove it not only oxidizes when in contact with an oxidizing atmosphere, but the formed oxide volatilizes very quickly, and at a corresponding rate as the temperature is increased. It is obvious that under such conditions molybdenum is very soon destroyed unless protected.

Various methods for protecting molybdenum, tungsten, alloys thereof with each other, and alloys thereof having approximately the oxidation properties of such metals, such as those with only small proportions of metal of the group consisting of cobalt, nickel and iron, have been proposed and tried. By the expression "alloys of molybdenum with small proportions of metal selected from the group consisting of cobalt, nickel, iron and tungsten," we mean such in which the proportion of any one of the

2

first three mentioned alloying metals is not greater than  $\frac{1}{2}\%$ , and in which the proportion of tungsten is not greater than 20%. In the same way the expression "alloys of tungsten with small proportions of metal selected from the group consisting of cobalt, nickel, iron and molybdenum," means such in which the proportion of any one of the first three mentioned alloying metals is not greater than  $\frac{1}{2}\%$  and in which the proportion of molybdenum is not greater than 20%. It will, however, be understood that our invention is also suitable for protecting alloys of molybdenum and tungsten in any proportion, with and without small proportions of alloying metals selected from the group consisting of cobalt, nickel and iron. In other words, our method is suitable for protecting any refractory readily oxidizable metal from oxidation at high temperatures.

At the present time, probably the most widely used protection for molybdenum is a coating of molybdenum silicide. Such a coating may be produced by vapor depositing a thin layer of silicon on the hot surface of molybdenum. It can also be formed by a painted or sprayed on and sintered method, or one such as described and claimed in the Garrison and Lovett application, Ser. No. 759,256, filed July 5, 1947; now patent No. 2,650,903, filed July 5, 1947, and owned by the assignee of the present application. While such a coating has very good protective value at elevated temperatures, its brittleness may result in cracking when struck or deformed. In order to be of value, any protective coating must completely cover the molybdenum or tungsten surface. Any defects, such as a crack or pinhole makes the coating useless since molybdenum, or other similar material, will erode by oxidation at the point of defect.

Other suggested methods of protection for molybdenum are the formation of alloys thereon, the application of ceramic coatings, and cladding. All of such methods however are very limited in application, and there is still a great need for protective coatings for molybdenum and the like.

In accordance with our invention, we employ electro-deposited coatings for the protection of metals of the class contemplated. Specifically, we propose a process whereby a black complex chromium base coating is applied electrolytically to the surface of the metal to be protected. Such a coating is preferably a chromium-vanadium or chromium-nickel-vanadium complex.

Before applying such a coating to a surface to be protected against oxidation, the same is thoroughly cleaned to remove any oil, grease, or contamination therefrom. This may be accomplished by methods now in general use for such purpose. However, a more thorough cleaning can be given, in addition to the above, by firing the molybdenum in a non-carburizing reducing atmosphere, such as is provided by hydrogen. Such a treatment produces a very clean active surface on molybdenum or other similar materials, as contemplated.

The clean molybdenum piece is made of the cathode 13 in an electrolytic cell, with the anode or anodes 14 made of lead, carbon, graphite, or other material which is insoluble when so used in chromium plating. Such a cell is represented in Fig. 1 of the drawing, which is now referred to specifically. In said figure, a container or tank 11 of material resistant to the action of the electrolyte, such as glass or other ceramic, is shown holding an electroplating bath 12 of a composition consisting of an aqueous solution of chromium trioxide (150 to 350 grams per liter) and a vanadium salt or salts (2 to 10 grams of vanadium per liter) so that there is present from 100 to 20 parts by weight of chromium per part of vanadium. Thus, a solution is desirably prepared from chromium trioxide ( $\text{CrO}_3$ )

and a vanadium salt or salts, in the ratio of about 20 parts chromium to about 1 part vanadium. Although any soluble vanadium salt, not including harmful material, may be employed, we prefer ammonium metavanadate. However, other soluble vanadium compounds, such as vanadium halide or the nitrate, may be substituted.

A typical solution contains chromium trioxide ( $\text{CrO}_3$ ), 200 grams per liter, ammonium metavanadate, 20 grams per liter, and glacial acetic acid, 6.5 ml. per liter. The acetic acid, or other soluble carboxylic acid, such as formic, citric, oxalic or propionic acid is added in a proportion of from 3 to 20 grams per liter to increase the working temperature range and obtain more uniform coatings.

Another electrolyte that can be used to produce such protective coatings contains chromium trioxide, nickel chloride, and a soluble vanadium salt, in an approximate ratio of 20 parts chromium to 4 parts nickel to 1 part vanadium. A typical solution contains chromium trioxide ( $\text{CrO}_3$ ), 200 grams per liter; nickel chloride ( $\text{NiCl}_2 \cdot 6\text{H}_2\text{O}$ ), 80 grams per liter; and 5 grams per liter of vanadium dissolved in just sufficient nitric acid to effect solution of the metal. To each liter of solution, 5 to 10 ml. of glacial acetic acid, or other soluble carboxylic acid, is added. Nickel sulfate is not a substitute for nickel chloride in such an electrolyte, as the sulfate radical produces inferior coatings.

After electroplating from one of the solutions before mentioned, a black uniform deposit is obtained upon the metal surface with a current-density of one ampere per square centimeter, and at a potential difference between the electrodes 13 and 14 of about 12 to 15 volts. The temperature of the bath is desirably maintained between 35° and 50° C., cooling coils (not shown) being used in the electrolyte, if necessary. The deposit on the cathode 13 consists of finely divided chromium metal, in a mixture of the oxides of chromium and vanadium or in a mixture of the oxides of chromium, nickel and vanadium and of finely divided nickel metal. Care must be taken that the deposit completely covers the surface of the material to be protected, with no pin-holes. The application of several layers insures complete coverage of the surface. The thickness of the deposited material 18, as shown in Fig. 2, of course depends on the length of time the plating is continued. A desirable thickness is from .001" to .005", which may be obtained in a period of from 5 to 25 minutes.

After plating, the oxidizable refractory metal has a protective coating on its surface, which is not only resistant to oxidation when heated in an oxidizing atmosphere, but it is also resistant to the action of nitric acid and many other chemical reagents, except hydrochloric acid by which it is slowly attacked.

Durability of the coating may be improved by firing in hydrogen for several hours at about 1200° C. An electric furnace, for this purpose, is illustrated at 15 in Fig. 3. In such a furnace the plated molybdenum or the like is heated in a stream of hydrogen, or other non-carburizing reducing or protective atmosphere in which hydrogen is the active ingredient, as by means of an electrical resistance element 16 surrounding a tube 17 of alumina to about 1200° C. for preferably several hours. The coated material 13 may be held in said furnace in a boat 19, of alumina or other inert refractory material, while subjected to the action of the reducing atmosphere.

After the firing in hydrogen or the like, additional layers of the coating can be applied, followed by another cycle of firing in the reducing atmosphere after the application of each layer. In this way the coating is at least partially diffused into the metal to be protected, thereby increasing its protective properties and bonding, and a dense protective coating is obtained. Molybdenum, for example, coated in this manner has been

fired in air at 1200° C. for several hours without any evident loss of molybdenum. The higher the temperature of the firing in hydrogen and the longer the duration of this firing, the more diffusion of the coating into the molybdenum occurs. The use to which the article is to be put determines whether it is permissibly fired at such temperatures.

Although preferred embodiments have been disclosed, it will be understood that modifications may be made within the spirit and scope of the invention.

We claim:

1. The method of protecting against oxidation at high temperatures articles constructed of metal of the group consisting of molybdenum, tungsten, and alloys thereof with each other and with small proportions of metal of the group consisting of cobalt, nickel and iron, comprising cleaning said articles, and electroplating by making them cathodes in an electrolytic cell with lead anodes, and in which the electrolyte consists of an aqueous solution of chromic acid containing 150 to 350 grams of chromium trioxide per liter and vanadium salt containing 2 to 10 grams of vanadium per liter, with a ratio of about twenty parts chromium to one part vanadium, said electrolyte also containing acetic acid to increase the working temperature range and obtain more uniform coatings, with a current density during plating of about one ampere per square centimeter, with a potential difference of about 12 to 15 volts, and a bath temperature of between 35° and 50° C., to produce thereon a chromium-vanadium complex.

2. The method of protecting against oxidation at high temperatures articles constructed of metal of the group consisting of molybdenum, tungsten, and alloys thereof with each other and with small proportions of metal of the group consisting of cobalt, nickel and iron, comprising cleaning said articles, electroplating by making them cathodes in an electrolytic cell with lead anodes, and in which the electrolyte consists of an aqueous solution of chromic acid containing 150 to 350 grams of chromium trioxide per liter and vanadium salt containing 2 to 10 grams of vanadium per liter, with a ratio of about twenty parts chromium to one part vanadium, said electrolyte also containing acetic acid to increase the working temperature range and obtain more uniform coatings, with a current density during plating of about one ampere per square centimeter, with a potential difference of about 12 to 15 volts, and a bath temperature of between 35° and 50° C., to produce thereon a chromium-vanadium complex, and firing in hydrogen for several hours at about 1200° C. to diffuse the coatings into the articles.

3. The method of protecting against oxidation at high temperatures articles constructed of metal of the group consisting of molybdenum, tungsten, and alloys thereof with each other and with small proportions of metal of the group consisting of cobalt, nickel and iron, comprising cleaning said articles, and electroplating by making them cathodes in an electrolytic cell in which the electrolyte consists of an aqueous solution of chromic acid containing 150 to 350 grams of chromium trioxide per liter, and vanadium salt containing 2 to 10 grams of vanadium per liter, said electrolyte also containing acetic acid to increase the working temperature range and obtain more uniform coatings, with a current density during plating of about one ampere per square centimeter, and a bath temperature of between 35° and 50° C., to produce thereon a chromium-vanadium complex.

4. The method of protecting against oxidation at high temperatures articles constructed of metal of the group consisting of molybdenum, tungsten, and alloys thereof with each other and with small proportions of metal of the group consisting of cobalt, nickel and iron, comprising cleaning said articles, electroplating by making them

cathodes in an electrolytic cell in which the electrolyte consists of an aqueous solution of chromic acid containing 150 to 350 grams of chromium trioxide per liter and vanadium salt containing 2 to 10 grams of vanadium per liter, said electrolyte also containing acetic acid to increase the working temperature range and obtain more uniform coatings, with a current density during plating of about one ampere per square centimeter, and a bath temperature of between 35° and 50° C., to produce thereon a chromium-vanadium complex, and firing in 10 hydrogen for several hours to diffuse the coatings into the articles.

5. The method of protecting against oxidation at high temperatures articles constructed of metal of the group consisting of molybdenum, tungsten, and alloys thereof with each other and with small proportions of metal of the group consisting of cobalt, nickel and iron, comprising cleaning said articles, and electroplating by making them cathodes in an electrolytic cell in which the electrolyte consists of an aqueous solution of chromic acid containing about 200 grams of chromium trioxide 15

5

10

20

per liter, nickel chloride containing about 80 grams  $\text{NiCl}_2 \cdot 6\text{H}_2\text{O}$  per liter, and vanadium salt containing about 5 grams of vanadium per liter, said electrolyte also containing acetic acid to increase the working temperature range and obtain more uniform coatings, with a current density during plating of about 1 ampere per square centimeter, and a bath temperature of between 35° and 50° C., to produce thereon a chromium-nickel-vanadium complex.

## References Cited in the file of this patent

## UNITED STATES PATENTS

|           |                 |       |               |
|-----------|-----------------|-------|---------------|
| 1,565,724 | Fonda           | ----- | Dec. 15, 1925 |
| 1,590,101 | Kyropoulos      | ----- | June 22, 1926 |
| 1,795,459 | Westbrook       | ----- | Mar. 10, 1931 |
| 1,975,239 | Ungelenk et al. | ----- | Oct. 2, 1934  |
| 2,144,250 | Allen et al.    | ----- | Jan. 17, 1939 |
| 2,304,297 | Anton           | ----- | Dec. 8, 1942  |
| 2,512,141 | Ma et al.       | ----- | June 20, 1950 |
| 2,555,372 | Ramage          | ----- | June 5, 1951  |
| 2,623,847 | Gilbert         | ----- | Dec. 30, 1952 |